

# UNITED STATES PATENT OFFICE.

FRANK C. MATHERS, OF BLOOMINGTON, INDIANA, ASSIGNOR TO AMERICAN SMELTING & REFINING CO., A CORPORATION OF NEW JERSEY.

## ELECTROLYTIC REFINING OF TIN.

1,397,222.

Specification of Letters Patent.

Patented Nov. 15, 1921.

No Drawing. Application filed October 11, 1918, Serial No. 257,700. Renewed December 9, 1920.  
Serial No. 429,561.

To all whom it may concern:

Be it known that I, FRANK C. MATHERS, a citizen of the United States, and resident of Bloomington, in the county of Monroe and State of Indiana, have invented certain new and useful Improvements in Electrolytic Refining of Tin, of which the following is a specification.

The invention relates in general to an improvement in the process of producing electrolytically refined tin from impure tin cast in the form of anodes and acted upon by an electrolyte and features the situation where there is a relatively low tin content and a relatively high sulfuric acid content.

Heretofore as disclosed in the patent to Robert L. Whitehead No. 1,157,830, dated October 26, 1915, it is proposed to produce from the impure tin which usually contains lead, antimony and other impurities, an electrolyte of such a character that it will insure the continued maintenance of the electrolytic decomposition of the tin during the refining operation. This Whitehead process consists fundamentally in maintaining at least a 6% solution of tin in the electrolyte and in this condition the process can be operated continuously when the electrolyte has in solution one-tenth of one per cent. sulfuric acid and 15-20% of hydrofluosilicic acid.

Difficulty is experienced with some grades of tin, such for instance as Bolivian tin which contains high percentages of impurities, when such metals are used to obtain and maintain the 6% solution of tin required by the Whitehead process. It takes time and power to practice the usual process to raise the baskets containing the tin shot into the electrolyte and even then, difficulty is experienced in obtaining such solution of tin as high as six per cent. The higher the percentage of tin required in the solution the more time is required at an increasing ratio and the greater is the difficulty of maintaining this high percentage and with some poor grades of tin it is practically impossible to maintain the 6% tin content after it has been initially obtained.

Accordingly, the primary object of the invention is to produce pure tin electrolytically from certain grades of impure tin anodes

with an electrolyte which is operative with a relatively low percentage of tin content.

Further due to present war conditions, the hydrofluosilicic acid required in the known process is difficult to obtain and has accordingly become somewhat expensive for extensive use in metallurgical processes. Economically, it is an advantage to reduce the amount of hydrofluosilicic acid but wherever attempts have been made to reduce the percentage of the hydrofluosilicic acid to any material extent below the 20% suggested in the Whitehead process, and especially where the tin content is as low as 2%, there resulted on the cathode plates the formation of projections and uneven coatings, called sprouts or trees, which gave rise to short circuits and other polarizing and deteriorating actions.

Accordingly, another object of the invention is to provide an electrolyte of the kind suggested and in which it is possible to reduce the amount of hydrofluosilicic acid used below what has heretofore been necessary, and at the same time to maintain the continuity of action during the electrolytic process free of polarizing and other objectionable results.

Broadly, I attain these objects by introducing a new addition agent to the usual electrolyte which agent permits of a reduction of the hydrofluosilicic acid content and at the same time causes the deposition of an unusually pure tin even when the electrolyte contains as low as 2% by weight tin in content.

Of the commercially available substances which are utilized as the addition agent, cresylic acid gives excellent results. A pure form of cresylic acid does not give as good results as the more or less impure commercial form and the best results have been obtained from the crude residue remaining in the still after the cresylic acid has been distilled out. This residue at present commands a high price and cannot be used commercially from an economical consideration. Certain other phenols have been used with satisfaction, fair results having been obtained by substances which consists of 40% of meta cresol; 35% of ortho cresol and 35%

of para cresol. Certain other substances, such for instance as benzol have been used and it is to be assumed that the beneficial agent is some substance common to all these 5 reagents.

Following the sequence of steps recited in the patented process above recited, the electrolyte particularly forming the novel element of this disclosure, is prepared from 10 impure tin anodes containing tin, copper, lead, or other material. As an example of one suitable type of electrolyte a solution of cresylic acid about  $\frac{3}{5}$  of 1%, hydrofluosilicic acid about 5 $\frac{1}{2}$ %, and sulfuric acid 5% by 15 weight has given satisfactory results. An electric current of suitable voltage and amperage is applied until upon testing the solution has taken up about 2% by weight of tin whereupon the passage of the current is 20 continued. During this formation of the electrolyte, the sulfuric acid contained in the solution combines with the lead and certain other impurities in accordance with known chemical reactions and precipitates certain 25 of the impurities which would otherwise go into solution as is well known in such processes. The electrolyte thus formed consists of tin dissolved in the hydrofluosilicic acid and presumably in the cresylic acid which 30 tin has been formed from the impure tin anodes without bringing any of the lead or other impurities into solution. The electrolyte thus formed is utilized as an electrolyte in the refining operation. The tin is 35 taken from the highly impure tin anodes and deposited on the cathodes in an unusually pure state. This cathode tin is characterized by hard, uniformly dense and crystalline structure; is free from projections and is 40 of substantially uniform thickness. It is commercially pure, testing over 99.9%. The tin thus formed is disclosed as a new composition of matter, which composition of matter is a pure grade of tin particularly 45 desirable for technical purposes and is of a higher grade than has been produced even from the high grade tin ores obtained from the Malay Straits Settlements. The process herein disclosed can be performed and the 50 product produced even from the highly impure grades of Bolivian and South American ores.

It is comparatively easy to obtain a 2% solution of tin and this is all that is necessary to obtain an operative electrolyte in the presence of the addition agent. It is noted that the amount of hydrofluosilicic acid is reduced from the necessary 20% recited in the Whitehead disclosure to about 5% and the process admits of the use of even a lower percentage of hydrofluosilicic acid. At the same time this process permits the use of a greater percentage of sulfuric acid than has been possible heretofore,

it being noted that higher percentages of acid may be used if necessary but this high percentage of sulfuric acid which would have been objectionable in the presence of the old twenty per cent. of hydrofluosilicic acid is not objectionable in the presence of the low tin percentage herein suggested.

In the preceding statement no reference has been made to the use of glue as an additional reagent in the electrolyte because the process has given satisfactory results 75 without the employment of glue. However, if a little glue is added together with the cresol even better results are attained and in the most perfected process the use of the usual amount of glue is suggested.

Having thus described my invention, I claim:—

1. In the electrolytic refining of impure tin, the process which consists in employing as the electrolyte a solution of tin in hydrofluosilicic acid, sulfuric acid and cresylic acid and in which the tin content is approximately two per cent. by weight.

2. In the electrolytic refining of impure tin, the process which consists in passing an electric current of suitable voltage and amperage from the tin anode to a cathode through an electrolyte solution containing cresylic acid and containing less than six per cent. by weight of tin in solution.

3. In the electrolytic refining of impure tin, the process which consists in passing an electric current of suitable voltage and amperage from the tin anode to a cathode through an electrolyte solution containing cresylic acid and containing approximately two per cent. by weight of tin in solution.

4. In the electrolytic refining of impure tin, the process which consists in passing an electric current of suitable voltage and amperage from the tin anode to a cathode through an electrolyte solution containing a solution of hydrofluosilicic acid, cresylic acid and less than six per cent. by weight of tin.

5. An electrolyte for the deposition of tin comprising an electrolyte solution of tin in hydrofluosilicic acid in the proportions approximately of two per cent. by weight of tin and five per cent. by weight of the free acid together with an addition agent capable of causing the tin to deposit in a coherent form when a suitable current is passed therethrough from an impure tin anode to a cathode.

6. In the electrolytic refining of impure tin the process of producing an appropriate electrolyte for the refining operation which consists in passing an electric current of suitable voltage and amperage from the impure tin as an anode to a cathode through a solution of hydrofluosilicic acid having a strength of less than 20% and in the pres-

- ence of an addition agent capable of preventing polarization and the production of trees on the cathode incidental to processes when there is a reduction in the 20% 5 strength of hydrofluosilicic acid used.
7. In the electrolytic refining of impure tin the process of producing an appropriate electrolyte for the refining operation which consists in passing an electric current of 10 suitable voltage and amperage from the impure tin as an anode to a cathode through a solution of hydrofluosilicic acid having a strength of less than 20% and in the presence of an addition agent capable of preventing polarization and the production of 15 trees on the cathode incidental to processes when there is a reduction in the 20% strength of hydrofluosilicic acid used and in the presence of sulfuric acid.
- 20 8. In the electrolytic refining of impure tin, the process of producing an appropriate electrolyte for the refining operation which consists in passing an electric current of suitable voltage and amperage from the impure tin as an anode to a cathode through a solution containing cresylic acid.
9. In the electrolytic refining of impure tin, the process of producing an appropriate electrolyte for the refining operation which 25 consists in passing an electric current of suitable voltage and amperage from the impure tin as an anode to a cathode through a solution containing cresylic acid in an impure form.
- 30 10. In the electrolytic refining of impure tin, the process of producing an appropriate electrolyte for the refining operation which consists in passing an electric current of suitable voltage and amperage from the impure tin as an anode to a cathode through a solution containing a phenol.
- 35 11. In the electrolytic refining of impure tin, the process of producing an appropriate electrolyte for the refining operation which 40 consists in passing an electric current of suitable voltage and amperage from the impure tin as an anode to a cathode through a solution of hydrofluosilicic acid having a strength of less than 20% and in the presence of an addition agent containing a phenol in the solution.
- 45 12. In the electrolytic refining of impure tin containing lead, the process of preventing contamination of the tin deposited from the impure tin anode upon the cathode, which 50 consists in employing as the electrolyte a solution of tin in hydrofluosilicic acid, together with a protective agent sufficient to convert the lead contained in the dissolving tin anode into a compound insoluble in the electrolyte and an addition agent capable of preventing polarization and the production of trees on the cathode.
- 55 13. In the electrolytic refining of impure tin containing lead, the process of preventing contamination of the tin deposited from the impure tin anode upon the cathode which 60 consists in employing as the electrolyte a solution of tin in hydrofluosilicic acid, together with a protective agent sufficient to convert the lead contained in the dissolving tin anode into a compound insoluble in the electrolyte and an addition agent containing a phenol.
- 65 14. In the electrolytic refining of impure tin containing lead, the process of preventing contamination of the tin deposited from the impure tin anode upon the cathode which 70 consists in employing as the electrolyte a solution of tin in hydrofluosilicic acid, together with a protective agent sufficient to convert the lead contained in the dissolving tin anode into a compound insoluble in the electrolyte and an addition agent containing a phenol.
- 75 15. A composition of matter constituting an electrolytically refined and chemically pure tin characterized by a hard, dense and finely crystalline structure.
- 80 16. An electrolytically produced cathode characterized by a hard, uniformly dense, crystalline structure, free from projections and of substantially uniform thickness.
- 85 17. In the electrolytic refining of impure tin, the process of producing an appropriate electrolyte for the refining operation which 90 consists in passing an electric current of suitable voltage and amperage from the impure tin as an anode to a cathode through a solution containing cresylic acid and glue.
- 95 18. In the electrolytic refining of impure tin, the process of producing an appropriate electrolyte for the refining operation which 100 consists in passing an electric current of suitable voltage and amperage from the impure tin as an anode to a cathode through a solution containing a phenol and glue.
- 105 19. In the electrolytic refining of impure tin containing lead, the process of preventing contamination of the tin deposited from the 110 impure tin anode upon the cathode which consists in employing as the electrolyte a solution of tin in hydrofluosilicic acid, together with a protective agent such as hydrofluosilicic acid of a strength sufficient to convert the lead contained in the dissolving tin anode into a compound insoluble in the electrolyte and an addition agent containing cresylic acid and glue.
- 115 20. In the electrolytic refining of impure tin, the process which consists in employing as the electrolyte a solution of tin, sulfuric and cresylic acids.
- 120 21. In the electrolytic refining of impure tin, the process of producing an appropriate electrolyte for the refining operation which 125 consists in passing an electric current of suitable voltage and amperage from the im-

pure tin as an anode to a cathode through with an addition agent capable of causing a solution containing a phenol sulfuric acid the tin to deposit in a coherent form when 10 and a tin dissolving agent.

22. An electrolyte for the deposition of tin 5 comprising an electrolyte solution of tin a free acid in the proportions approximately of two per cent. by weight of tin and five per cent. by weight of the free acid together

with an addition agent capable of causing the tin to deposit in a coherent form when 10 a suitable current is passed therethrough from an impure tin anode to a cathode.

Signed at Bloomington, in the county of Monroe and State of Indiana, this 27th day of Sept., A. D. 1918.

FRANK C. MATHERS.